# EUROPEAN PATENT SPECIFICATION

(11) **EP 0 412 788 B1**
(45) Date of publication and mention of the grant of the patent: **12.01.1994**
(21) Application number: 90308707.0
(22) Date of filing: 08.08.1990
(51) Int. Cl.: C10M 173/02

(54) **Lubrication method for cold plastic working of metallic materials**
Schmierverfahren zur plastischen Bearbeitung metallischer Materialien
Méthode de lubrification pour traitement de matériaux métalliques lors du travail plastique à froid

(30) Priority: 09.08.1989 JP 204585/89
(43) Date of publication of application: 13.02.1991
(73) Proprietor: NIHON PARKERIZING CO., LTD., Chuo-ku Tokyo 103 (JP)
(72) Inventor: Fujii, Hiroyuki, c/o Nippondenso Co.,Ltd., Kariya-City, Alchi-Pref, 448 (JP); Mizutani, Takanori, c/o Nippondenso Co.,Ltd., Kariya-City, Alchi-Pref, 448 (JP); Shirai, Tokuo, c/o Nippondenso Co.,Ltd., Kariya-City, Alchi-Pref, 448 (JP); Nagae, Yoshio, c/o Nihon Parkerizing Company, Ltd., Tokyo (JP); Kaburaki, Kouji, c/o Nihon Parkerizing Company,Ltd, Tokyo (JP); Hetsugi, Kouji, c/o Nihon Parkerizing Company, Ltd, Tokyo (JP); Tanizawa, Yasuo, c/o Nihon Parkerizing Company,Ltd, Tokyo (JP)
(74) Representative: Hale, Stephen Geoffrey

(56) References cited:
- EP-A- 0 261 438
- EP-A- 0 270 836
- DE-A- 1 030 495
- DE-A- 3 922 464
- FR-A- 2 102 283
- US-A- 4 148 970
- US-A- 4 303 537

## Description

### BACKGROUND OF THE INVENTION

### 1. Field of the Invention

This invention relates to a lubrication method for cold plastic working metallic materials using an aqueous treatment liquid.

More particularly, this invention relates to the cold plastic working (forging, tube drawing, wire drawing, etc.) of metallic materials, for example, steel, stainless steels, titanium-based alloys, copper, copper-based alloys, aluminum and aluminum-based alloys, using an aqueous lubrication treatment liquid).

### 2. Description of the Related Arts

As aqueous lubrication treatment liquids currently used for the cold plastic working of a metallic material, liquids which comprise a solid lubricant, for example, molybdenum disulfide or graphite, at least one member selected from inorganic binders and organic binders, and a surfactant are known.

When a cold working is carried out at a relatively small reduction, a method in which an aqueous lubrication treatment liquid is brought directly into contact with a surface of a metallic material free from grease, followed by drying to form a solid lubricant film thereon, is known.

In a high reduction cold working, a method is employed of forming a solid lubricant film over a chemical conversion coating where a metallic material surface, after the formation of the chemical conversion coating, is brought into contact with an aqueous lubrication treatment liquid, followed by drying, or has a solid lubricant powder deposited thereon. Using a solid lubricant in a powder state, however, causes a problem of a deterioration of the working environment, and thus most preferably a lubricant in the form of an aqueous treatment liquid is used. In this case, however, a conventional aqueous lubricant treatment liquid has a drawback in that it has an unstable and insufficient lubricating property and causes rusting of the treated or formed metallic material when left to stand after the lubricating treatment or a plastic working.

In the above cases, the currently used treatment agents cannot provide a stable and desired lubricity, which often results in the problems of seizing and galling.

US-A-4,303,537 discloses an aqueous lubricant for the treatment of metallic surfaces, the lubricant comprising molybdenum disulfide and graphite, for example in amounts of 15 to 30%, and an acrylic resin.

US-A-4,148,970 discloses an aqueous lubricant composition for application to metal surfaces to hinder primer removal during metal formation, the lubricant comprising a metallic stearate, an emulsifier, titanium dioxide (typically provided in the form of a pigment useful in the paint art in a condition such that it will readily disperse in water, advantageously less than about 200 mesh (US sieve series)), and Xanthomonas hydrophilic colloid.

DE-A-1,030,495 discloses an aqueous lubricant for cold working metallic surfaces, the lubricant comprising zinc stearate, talc and an emulsifier.

### SUMMARY OF THE INVENTION

An object of the present invention is to provide a lubrication method for cold plastic working metallic materials using an aqueous treatment liquid which does not have the above-mentioned disadvantages of conventional aqueous lubrication treatment liquids and exhibits a high stability and an excellent lubricating property, without causing a rusting of the metallic materials.

The above-mentioned object can be attained by a lubrication method which comprises treating the metallic material with an aqueous lubrication treatment liquid for cold plastic working metallic materials, which liquid comprises 4 to 160 g/l of a metallic soap, 50 to 400 g/l of a solid lubricant as hereinafter specified, 0.5 to 40 g/l of a surfactant for uniformly dispersing the metallic soap and the solid lubricant, a colloidal titanium compound as hereinafter specified in an amount of 10 to 5000 ppm expressed in terms of titanium, and water.

The aqueous lubrication treatment liquid used in the present invention optionally further comprises 5 to 150 g/l of a binder.

### DESCRIPTION OF THE PREFERRED EMBODIMENTS

The inventors of the present invention found for the first time that a lubricating film having an excellent lubricating activity not obtained by the conventional aqueous lubrication treatment liquid and a superior resistance to rust on a surface of metallic article, for example a cold plastic processed steel article, can be formed on a surface of a metallic article by applying an aqueous lubrication treatment liquid comprising in specified amounts a metallic soap, a solid lubricant of specified type, a surfactant and a colloidal titanium compound of specified type.

Furthermore, the inventors of the present invention found that, in the above-mentioned aqueous lubrication treatment liquid, an addition of a binder to the metallic soap, solid lubricant, surfactant, and colloidal titanium compound is effective for further enhancing the lubricating property thereof, due to the synergistic effect of the binder with the other components, for example, the metallic soap and the colloidal titanium compound.

The present invention was completed based on the above-mentioned findings.

The aqueous lubrication treatment liquid for use in the present invention comprises, as principal components, 4 to 160 g/l of a metallic soap, 50 to 400 g/l of a solid lubricant as hereinafter specified, 0.5 to 40 g/l of a surfactant for uniformly dispersing the metallic soap and the solid lubricant in water, 10 to 5000 ppm expressed as titanium of a colloidal titanium compound as hereinafter specified, and water.

The metallic soap usable for the present invention preferably comprises at least one member selected from salts of fatty acids and hydroxy-fatty acids having 12 to 22 carbon atoms with multivalent metals. The fatty acids and the hydroxy-fatty acids usable for the present invention include lauric acid, myristic acid, palmitic acid, stearic acid, behenic acid and hydroxystearic acids. A preferable fatty acid is stearic acid. The multivalent metals usable for the present invention are preferably selected from calcium, aluminum, magnesium, barium and zinc.

A particularly preferable metallic soap for the present invention is a wet state calcium stearate prepared in accordance with JP-B 60-45680.

The metallic soap is contained in a dry content of 4 to 160 g/l, preferably 10 to 50 g/l, in the aqueous lubrication treatment liquid. If the metallic soap is employed in an amount of less than 4 g/l, the resultant lubricating film on a metallic article exhibits an unsatisfactory lubricating effect. Also, even if the content of the metallic soap is increased to a level above 160 g/l, the lubricating effect of the resultant lubricating film on a metallic article is substantially not increased higher than that resulted from 160 g/l of the metallic soap; rather the lubricating effect of the solid lubricant is restricted by the large amount of the metallic soap.

The solid lubricant usable for the present invention comprises at least one member selected from molybdenum disulfide, graphite, tungsten disulfide, fluorinated graphite, boron nitride and talc.

The content of the solid lubricant in the treatment liquid is 50 to 400 g/l, preferably 150 to 250 g/l. A content of the solid lubricant of less than 50 g/l does not provide a sufficient formation of a solid lubricating film on the metallic article surface. If the content of the solid lubricant is more than 400 g/l, the lubrication effect becomes saturated so that no further improvement of the lubrication effect is obtained, and the cost of the aqueous lubrication liquid is increased.

In the lubrication method of the present invention, when the metallic soap is employed in a mixing weight ratio of from 2:5 to 1:50 to the solid lubricant in the aqueous lubrication treatment liquid, the resultant lubricating film on the metallic article exhibits an excellent lubricating effect.

In the aqueous lubrication treatment liquid a surfactant is employed for dispersing the metallic soap and solid lubricant in water. There is no specific limitation of the type thereof.

Surfactants in general use include nonionic type surfactants, for example polyoxyethylene alkyl ethers, polyoxyethylene alkylphenyl ethers, polyoxyethylene alkyl esters, and polyoxyethylene sorbitane alkyl esters; anionic type surfactants, for example fatty acid salts, alkyl sulphates, alkyl sulphonate, alkyl phosphates and alkyl dithiophosphates; cationic type surfactants, for example aliphatic amine salts, and quarternary ammonium salts; and amphoteric type surfactants, for example amino acid type and betain type carboxylic acid salts, sulfuric ester salts, sulphonic ester salts, and phosphoric ester salts.

The content of the surfactant in the aqueous lubrication liquid for use in the present invention is 0.5 to 40 g/l, preferably 5 to 10 g/l. The content of the surfactant in the aqueous lubrication treatment liquid is preferably increased or decreased in response to the content of the solid lubricant. Where the content of surfactant is less than 0.5 g/l, the solid surfactant in the treatment liquid is insufficiently wetted, and a greater quantity than 40 g/l does not increase the dispersing effect of the surfactant to any significant degree.

The aqueous lubrication treatment liquid can be supplemented with another additive, for example, a high molecular dispersing agent, defoaming agent, and rust-preventive additive.

The aqueous lubrication treatment liquid also contains a colloidal titanium compound which is a neutralised reaction product of at least one member selected from compounds of sulphuric acid with titanium and compounds of phosphoric acid with titanium, said product being neutralised with an alkali, for example caustic soda or the like. The content of colloidal titanium in the aqueous lubrication treatment liquid is 10 to 5000 ppm, more preferably 50 to 300 ppm, expressed in terms of titanium.

When the colloidal titanium compound is employed in an amount of less than 10 ppm, the improvement in the lubricating effect and the rust-preventing effect of the resultant lubricating film on the metallic article surface is not significant. When the colloidal titanium compound is added in an amount of 10 ppm or more, however, the improvement in the lubricating effect and the rust-preventing effect of the resultant lubricating film becomes significant and increases with an increase in the content thereof. Accordingly, it is possible to increase the content of colloidal titanium compound to a high level, up to 5000 ppm as long as the preparation of the aqueous lubrication treatment liquid is possible.

The colloidal titanium compound usable for the present invention is in the form of colloidal particles consisting of negatively charged micelles. Accordingly, the colloidal titanium compound is definitely distinct from fine particles of titanium compounds, for example, titanium dioxide, usable for pigments, which particles are produced by finely pulberizing grains of the compounds, and the resultant particles do not have an electrical charge when dispersed in water.

The aqueous lubrication treatment liquid optionally contains a binder in addition to the above-mentioned components.

The binder preferably comprises at least one member selected from inorganic and organic binder materials and is effective for further enhancing the lubricating effect of the resultant lubricating film on the metallic article surface.

The inorganic binder is not restricted to a specific type of binder and preferably comprises at least one member selected from the borates, phosphates, and silicates mentioned below.
a. Borates
   Alkali metal salts, alkali earth metal salts and ammonium salts of HBO₂ , H₃BO₃ , H₄B₂O₅ , H₂B₄O₇ , HB₅O₈ , H₂B₆O₁₀ , H₂B₈O₁₃ , etc.
b. Phosphates
   Alkali metal salts, alkali earth metal salts and ammonium salts of H₃PO₄ , HPO₃ , H₄P₂O₆ , H₃PO ₃ , H₄P₂O₅ , HPO₂ , H₃PO₂ , H₃P₃O₉ , and polyphosphoric acids, for example, H₄P₂O₇ , H₅P₃O₁₀ , H₆P₁₁O₁₃ , etc.
c. Silicates
   Those expressed by the general formula M₂O.XSiO₂ , where M denotes an alkali metal atom or alkali earth metal atom and x denotes a positive integer of 1 to 5.

The organic binder is not limited to a specific type of binder, and preferably comprises at least one member selected from water-soluble high molecular compounds, for example, natural high molecular substance much as starch, sea weeds, vegetable mucilages, animal proteins, and fermentation mucilages; semi-synthetic high molecular substances prepared from starch and cellulose; and synthetic polymers, for example, polyvinyl pyrrolidone, polyethylene glycol, and polyvinyl alcohol.

The binder is employed in a solid content of 5 to 150 g/l, preferably 10 to 50 g/l, in the aqueous lubrication treatment liquid for use in the present invention. This solid content is variable depending on the content of the solid lubricant. If the content of the binder is less than 5 g/l, the improvement in the bonding property of the resultant lubricating film to the metallic article surface is not satisfactory. Also, if the binder is employed in a too large content of more than 150 g/l, the resultant aqueous lubrication treatment liquid exhibits an undesirable high viscosity, and thus the amount of the aqueous lubrication treatment liquid adhered to the surface of the metallic article becomes too large. This large amount of the resultant lubricating film formed on the metallic article surface causes the metallic die, through/which the metallic article is cold plastic worked, to be clogged.

The aqueous lubrication treatment liquid for use in the present invention can be prepared by dispersing and dissolving the above-mentioned components in predetermined amounts in water in the same way as usually practiced.

When the total content of the components is relatively low, the resultant prepared liquid can be directly used as an aqueous lubrication treatment liquid. If the total content of the components is relatively high, the resultant prepared liquid is directly used or diluted with an additional amount of water and then used as an aqueous lubrication treatment liquid, in response to the type of metallic article, the type of cold plastic working, and the intensity of the working.

The metallic article to be treated by the aqueous lubrication treatment liquid is optionally subjected to a chemical conversion procedure before the lubrication treatment.

There is no specific restriction of the type of the chemical conversion layer on the metallic material, and, for example, zinc phosphate treatment, iron oxalate treatment, cuprous oxide treatment, aluminum fluoride treatment, and titanium fluoride treatment commonly used according to the type of metals, can be used.

The aqueous lubrication treatment liquid for use in the present invention is applied to a metallic material, usually by an immersion procedure wherein the temperature thereof is maintained at a level between room temperature and 80°C.

When the aqueous lubrication treatment liquid is applied at a high temperature, the metallic article is also heated, and thus the layer of the aqueous lubrication treatment liquid formed on the metallic article surface can be dried at an enhanced drying efficiency. Nevertheless, if the temperature of the aqueous lubrication treatment liquid becomes too high, the viscosity and concentration of the aqueous lubrication treatment liquid is altered, and thus a complicated control becomes necessary to maintain the viscosity and concentration of the aqueous lubrication treatment liquid at a predetermined level by supplying water thereto.

The lubrication process of the present invention usually is carried out in one of the following sequences. The sequence is variable depending on the type of metallic article, surface condition, type of cold plastic working, and grade of reduction.
① Degreasing - water rinsing - lubrication treatment according to the present invention - drying
② Degreasing - water rinsing - pickling - water rinsing - lubrication treatment according to the present invention - drying (pickling is carried out to remove rust and scale)
③ Degreasing - water rinsing - pickling - water rinsing -chemical conversion treatment - water rinsing - lubrication treatment according to the present invention - drying
④ Degreasing - water rinsing - chemical conversion treatment - water rinsing - lubrication treatment according to the present invention - drying

The degreasing is optionally carried out when necessary. The pickling is carried out to remove rust and scale from the metallic article surface.

The metallic article is optionally surface-treated by a shot blast treatment or a sand blast treatment or by the above-mentioned chemical conversion procedure, before the lubrication treatment. The type of surface treatment can be chosen in consideration of the type and surface condition of the metallic article, and the type and intensity of the cold plastic working procedure.

By applying the specific aqueous lubrication treatment liquid in accordance with the present invention, the resultant solid lubricating film formed on the metallic article surface or on the chemical conversion layer exhibits an excellent lubricating effect and rust-preventive effect in comparison with that derived from the conventional aqueous lubrication treatment liquid.

The present invention offers a lubrication method for cold plastic working of metallic articles by which the metallic articles can be given an excellent lubricating property that enables a satisfactory high reduction of a cold plastic working without seizure and galling, with a high workability, and giving the thus processed products a high rust resistance.

### EXAMPLES

The present invention will be further explained by way of Examples and Comparative Examples, which in no way limit this invention.

### Examples 1 - 13 and Comparative Examples 1 - 19

In each of these Examples and comparative Examples, a bar consisting of a carbon steel (JIS G4051) and having a diameter of 30 mm was subjected to the following procedures.

Degreasing → water rinsing → pickling → water rinsing → chemical conversion treatment → water rinsing → lubrication treatment → drying

In the degreasing stage, the carbon steel bar was treated in a solution containing 20 g/l of Fine Cleaner 4360 (trademark of degreasing agent, a product of Nihon Parkerizing Co.) at 70°C for 10 min.

In each water rinse stage, the carbon steel bar was treated with running city water at room temperature for 60 sec.

The pickling procedure was carried out by using an Ivit 700 A (trademark: made by Asahi Kagaku K.K.) in an amount of 0.05 g/l at room temperature for 10 minutes.

The chemical conversion procedure was carried out by immersing the carbon steel bar in an aqueous solution containing a zinc phosphate type chemical conversion film-forming agent (trademark: PB181X, made by Nihon Parkerizing K.K.) in an amount of 90 g/l. An accelerator for the chemical conversion film-forming agent (trademark: AC131, made by Nihon Parkerizing K.K.) was applied in an amount of 0.3 g/l at a temperature of 80°C for 15 minute, except for Examples 12 and 13 and Comparative Examples 7,8,9 and 15, wherein the chemical conversion was not applied.

The lubrication treatment was carried out by immersing the carbon steel bar in the aqueous lubrication treatment liquid having the composition as shown in Table 1 at a temperature of 80°C for 3 minutes, except for Comparative Examples 6 and 11, and the treatment was carried out at a temperature of 70°C for 3 minutes.

The drying procedure was carried out by blowing hot air at a temperature of 120°C for 10 minutes. Usually, the dying procedure can be carried out by leaving the treated metallic article to stand in the ambient atmosphere.

The resultant lubrication treated carbon steel bar was subjected to the cold forging test (cold backward cup extrusion test) as indicated in Table 2.

The lubricating effect was evaluated by measuring a largest depth of a good inner surface of the extruded cup which could be formed without generating galling or fouling in the form of vertical lines on the inside wall surface of the extruded cup. The greater the deepest depth of the good inner surface of the cup, the better the lubricating effect of the resultant lubricating film on the bar surface.

The test results are indicated in Table 1.

Also, the lubrication treated carbon steel bar was subjected to the rust-resistance test as indicated in Table 3. The rust-resistance was evaluated in the following four classes.

The test results are indicated in Table 1.

In view of Table 1, in Comparative Examples 1 to 8 wherein the lubrication treatment liquid comprised the metallic soap, solid lubricant and surfactant and was free from the colloidal titanium compound, the resultant cup depth of the good inner surface was in the range of 30 to 48 mm and greater than that of Comparative Examples 9 to 13, in which the content of the metallic soap was at a low level of 4 g/l or less and in Comparative Examples 10 and 14 in which the content of the solid lubricant was less than 50 g/l. Accordingly, it is clear that the use of higher amounts of metallic soap and solid lubricant in the aqueous lubricant treatment liquids for use in the present invention provide an improved lubricating effect on the metallic article even the absence of the colloidal titanium compound.

In Comparative Examples 2 to 6, in which the aqueous lubrication treatment liquids contained 5 g/l or more of a binder, the resultant cup depth of the good inner surface was in the range of 34 to 38 mm and larger than the 32 mm of that in Comparative Example 1, in which no binder was employed. Therefore, it is clear that the addition of the binder effectively further enhances the lubricating effect of the aqueous lubrication treatment liquid.

In Examples 1 to 13 in which the aqueous lubrication treatment liquids contained a colloidal titanium compound, the resultant cup depth of the good inner surface was in the range of 36 to 54 mm, which is larger than that of the 30 to 48 mm in Comparative Examples 1 to 8 in which the colloidal titanium compound was not employed. Therefore, it is clear that the addition of the colloidal titanium compound effectively enhances the lubricating effect of the aqueous lubrication treatment liquid when used in the present invention.

In Comparative Example 15, in which the solid lubricant is in a low content of less than 50 g/l, and in Comparative Examples 16 and 18 in which colloidal titanium compound is in the low content of less than 10 ppm, the resultant cup depth of the good inner surface was in the range of 16 to 32 mm, and was unsatisfactory.

Further, in Examples 7 to 11, in which a binder was employed, the resultant cup depth of the good inner surface was 40 to 54 mm, which was larger than the 36 to 4 mm in Examples 1 to 6 in which no binder was employed. Therefore, it is clear that the addition of a binder effectively enhances the lubricating effect of the aqueous lubrication treatment liquid when used in the present invention.

In Examples 12 and 13, in which the chemical conversion was not applied, the resultant lubricating effect was a little lower than that in Examples 7 and 8 in which the chemical conversion was applied, but was higher than that in Comparative Example 19 in which a conventional aqueous lubrication treatment liquid was employed.

In Comparative Examples 1 to 8 and 9 to 14, in which the colloidal titanium compound was not employed, the resultant rust resistance was unsatisfactory (class 1 or 2), whereas in Examples 1 to 13 in which the colloidal titanium compound was employed, the resultant rust resistance was satisfactory (class 3 or 4). Accordingly, it is clear that the addition of the colloidal titanium compound effectively enhances the rust-preventive effect of the aqueous lubrication treatment liquid when used in the present invention.

### Examples 14 to 17 and Comparative Examples 20 to 29

In each of Examples 14 to 17 and Comparative Examples 20 to 29, the same procedures as those in Examples 1 were carried out, with the following exceptions.

The metallic article to be treated was a 13Cr stainless steel bar (SUS 410L, JIS G4303) having a diameter of 30 mm.

The pickling was carried out by using an aqueous solution of 7% of HNO₃ and 3% of HF at room temperature for 10 minutes.

The chemical conversion treatment was carried out by immersing the stainless steel bar in an aqueous solution containing 40 g/l of an oxalate type chemical conversion film-forming agent (trademark: FBA1, made by Nihon Parkerizing K.K.), 20 g/l of an oxalate type chemical conversion film-forming additive (trademark: FBA2, made by Nihon Parkerizing K.K.), and 1 g/l of an oxalate type chemical conversion film-forming accelerator (trademark: AC-16, made by Nihon Parkerizing K.K.) at a temperature of 90°C for 15 minutes.

The lubrication treatment was carried out by immersing the stainless steel bar in an aqueous lubrication treatment liquid having the composition as shown in Table 4, at a temperature of 80°C for 3 minutes, except that in Comparative Examples 14 and 18 the immersion treatment was carried out at a temperature of 70°C for 3 minutes.

The treated stainless steel bar was subjected to the cold forging test as indicated in Table 2.

The test results are shown in Table 4.

In Comparative Examples 20 to 22 using an aqueous lubrication treatment liquid free from the colloidal titanium compound, the depth of the good inner surface of cup was 38 to 54 mm, which is larger than the 28 to 32 mm in Comparative Examples 23 to 25. Accordingly, it is clear that, when applied to a stainless steel article, aqueous lubrication treatment liquids containing amounts of metallic soap and solid lubricant required by the invention exhibit a lubricating effect not obtained by the conventional lubrication treatment liquid.

In Examples 14 to 17 in which the colloidal titanium compound was employed, the depth of the good inner surface of cup was 44 to 58 mm, which is larger than the 28 to 32 mm in Comparative Examples 26 to 29 in which the contents of the metallic soap and solid lubricant fall outside of the scope of the present invention.

Also, it is clear that the lubricating effect of the aqueous lubrication treatment liquids in Examples 14 to 27, in which the colloidal titanium compound was added, is higher than that in Comparative Examples 20 to 22 in which the colloidal titanium compound was not employed.

### Examples 18 to 21 and Comparative Examples 30 to 33

In each of Examples 18 to 21 and Comparative Examples 30 to 33, the same procedures as those in Example 1 were carried out, with the following exceptions.

The metallic article to be treated was a titanium wire (Second type, JIS H4600) having a diameter of 3 mm.

The pickling was carried out by using an aqueous solution containing 7% of HNO₃ and 3% of HF at room temperature for 10 minutes.

The chemical conversion treatment was carried out by immersing the titanium wire in an aqueous solution containing 36 g/l of a fluoride type chemical conversion film-forming agent (trademark: MET-3851, made by Nihon Parkerizing K.K.) at a temperature of 60°C for 3 minutes.

The lubrication treatment was carried out by immersing the titanium wire in an aqueous lubrication treatment liquid having the composition as indicated in Table 5 at a temperature of 80°C for 3 minutes, except that, in Comparative Example 33, the treatment temperature was 70°C.

The resultant treated titanium wire was subjected to the cold wire drawing test as indicated in Table 6.

The test results are shown in Table 5.

Table 5 clearly indicates that, in Examples 18 to 21 in accordance with the present invention, the resultant lubrication treated titanium wires exhibited a high resistance to galling even after five passes of the cold drawing test whereas, in Comparative Examples 30 to 33, the resultant lubrication treated titanium wire had galls at the fifth pass of the cold drawing test.

## Claims

1. A lubrication method for a cold plastic working of a metallic material, which method comprises treating the metallic material with an aqueous lubrication treatment liquid comprising:
(a) 4 to 160 g/l of a metallic soap;
(b) 50 to 400 g/l of a solid lubricant consisting of at least one member selected from molybdenum disulfide, graphite, tungsten disulfide, fluorinated graphite, boron nitride and talc;
(c) 0.5 to 40 g/l of a surfactant for uniformly dispersing the metallic soap and the solid lubricant;
(d) a colloidal titanium compound which is a neutralised reaction product of at least one member selected from compounds of titanium with sulphuric acid and compounds of titanium with phosphoric acid, said product being neutralised with an alkali, and which is present in an amount of 10 to 5000 ppm expressed in terms of titanium; and
(e) water.

2. A method as claimed in claim 1, wherein the metallic soap comprises at least one member selected from salts of calcium, aluminum, magnesium, barium and zinc with fatty acids and hydroxy fatty acids having 12 to 22 carbon atoms.

3. A method as claimed in claim 2, wherein the acids for the metallic soap are selected from lauric acid, myristic acid, palmitic acid, stearic acid, behenic acid and hydroxystearic acid.

4. A method as claimed in any one of claims 1 to 3, wherein the metallic soap is present in a weight ratio of from 2:5 to 1:50 to the solid lubricant.

5. A method as claimed in any one of claims 1 to 4, wherein molybdenum disulfide is used as the solid lubricant, preferably in an amount of from 150 to 250 g/l.

6. A method as claimed in any one of claims 1 to 5, wherein the colloidal titanium compound is prepared by neutralizing titanium phosphate with caustic soda.

7. A method as claimed in any one of claims 1 to 6, wherein the colloidal titanium compound is present in an amount of at least 50 ppm.

8. A method as claimed in any one of claims 1 to 7, wherein the metallic material treated is a material having a chemical conversion coating layer formed thereon, and said layer is treated with the aqueous lubrication treatment liquid.

9. A method as claimed in any one of claims 1 to 8, wherein the aqueous lubrication treatment liquid further comprises 5 to 150 g/l of a binder.

10. A method as claimed in claim 9, wherein the binder comprises at least one member selected from inorganic borates, phosphates and silicates and water-soluble organic high molecular substances.

## Patentansprüche

1. Schmierverfahren zum Kaltverformen eines metallischen Materials, wobei das Verfahren umfaßt Behandeln des metallischen Materials mit einer wässerigen Schmierbehandlungsflüssigkeit, umfassend:
(a) 4 bis 160 g/l einer Metallseife;
(b) 50 bis 400 g/l eines festen Schmiermittels, bestehend aus mindestens einem Mitglied, ausgewählt aus Molybdändisulfid, Graphit, Wolframdisulfid, fluoriertem Graphit, Bornitrid und Talkum;
(c) 0,5 bis 40 g/l eines Tensids zum gleichförmigen Dispergieren der Metallseife und des festen Schmiermittels;
(d) eine kolloidale Titanverbindung, die ein Neutralisationsreaktionsprodukt von mindestens einem Mitglied, ausgewählt aus Verbindungen von Titan mit Schwefelsäure und Verbindungen von Titan mit Phosphorsäure ist, wobei das Produkt mit einem alkalischen Stoff neutralisiert wird und in einer Menge von 10 bis 5000 ppm, ausgedrückt als Titan, vorliegt; und
(e) Wasser.

2. Verfahren nach Anspruch 1, wobei die Metallseife mindestens ein Mitglied, ausgewählt aus Salzen von Calcium, Aluminium, Magnesium, Barium und Zink mit Fettsäuren und Hydroxyfettsäuren mit 12 bis 22 Kohlenstoffatomen umfaßt.

3. Verfahren nach Anspruch 2, wobei die Säuren für die Metallseife ausgewählt sind aus Laurinsäure, Myristinsäure, Palmitinsäure, Stearinsäure, Behensäure und Hydroxystearinsäure.

4. Verfahren nach einem der Ansprüche 1 bis 3, wobei die Metallseife in einem Gewichtsverhältnis von 2:5 bis 1:50 des festen Schmiermittels vorliegt.

5. Verfahren nach einem der Ansprüche 1 bis 4, wobei Molybdändisulfid als festes Schmiermittel verwendet wird, vorzugsweise in einer Menge von 150 bis 250 g/l.

6. Verfahren nach einem der Ansprüche 1 bis 5, wobei die kolloidale Titanverbindung durch Neutralisieren von Titanphosphat mit Natriumhydroxid (Ätznatron) hergestellt wird.

7. Verfahren nach einem der Ansprüche 1 bis 6, wobei die kolloidale Titanverbindung in einer Menge von mindestens 50 ppm vorliegt.

8. Verfahren nach einem der Ansprüche 1 bis 7, wobei das behandelte metallische Material ein Material ist mit einer chemischen Umwandlungsschicht darauf gebildet, und die Schicht mit der wässerigen Schmierbehandlungsflüssigkeit behandelt wird.

9. Verfahren nach einem der Ansprüche 1 bis 8, wobei die wässerige Schmierbehandlungsflüssigkeit zusätzlich 5 bis 150 g/l eines Bindemittels umfaßt.

10. Verfahren nach Anspruch 9, wobei das Bindemittel mindestens ein Mitglied, ausgewählt aus anorganischen Boraten, Phosphaten und Silicaten und wasserlöslichen organischen hochmolekularen Stoffen umfaßt.

## Revendications

1. Procédé de lubrification pour le travail à froid à l'état plastique d'un matériau métallique, ce procédé comprenant le traitement du matériau métallique avec un liquide aqueux de traitement de lubrification comprenant :
(a) 4 à 160 g/l d'un savon métallique;
(b) 50 à 400 g/l d'un lubrifiant solide constitué d'au moins un composé choisi parmi le disulfure de molybdène, le graphite, le disulfure de tungstène, le graphite fluoré, le nitrure de bore et le talc;
(c) 0,5 à 40 g/l d'un tensioactif servant à disperser uniformément le savon métallique et le lubrifiant solide;
(d) un composé de titane colloïdal qui est un produit de réaction neutralisé d'au moins un composé choisi parmi les composés du titane avec de l'acide sulfurique et les composés du titane avec de l'acide phosphorique, ledit produit étant neutralisé avec une base et étant présent en une quantité de 10 à 5 000 ppm, exprimée en termes de titane; et
(e) de l'eau.

2. Procédé selon la revendication 1, dans lequel le savon métallique comprend au moins un composé choisi parmi les sels de calcium, d'aluminium, de magnésium, de baryum et de zinc avec des acides gras et des hydroxyacides gras comportant de 12 à 22 atomes de carbone.

3. Procédé selon la revendication 2, dans lequel les acides servant à former le savon métallique sont choisis parmi l'acide laurique, l'acide myristique, l'acide palmitique, l'acide stéarique, l'acide béhénique et l'acide hydroxystéarique.

4. Procédé selon l'une quelconque des revendications 1 à 3, dans lequel le savon métallique est présent dans une proportion pondérale de 2 : 5 à 1 : 50 par rapport au lubrifiant solide.

5. Procédé selon l'une quelconque des revendications 1 à 4, dans lequel du disulfure de molybdène est utilisé comme lubrifiant solide, de préférence en une quantité de 150 à 250 g/l.

6. Procédé selon l'une quelconque des revendications 1 à 5, dans lequel le composé de titane colloïdal est préparé par neutralisation de phosphate de titane avec de la soude caustique.

7. Procédé selon l'une quelconque des revendications 1 à 6, dans lequel le composé de titane colloïdal est présent en une quantité d'au moins 50 ppm.

8. Procédé selon l'une quelconque des revendications 1 à 7, dans lequel le matériau métallique traité est un matériau sur lequel est formée une couche de revêtement de conversion chimique et ladite couche est traitée avec le liquide aqueux de traitement de lubrification.

9. Procédé selon l'une quelconque des revendications 1 à 8, dans lequel le liquide aqueux de traitement de lubrification comprend en outre 5 à 150 g/l d'un liant.

10. Procédé selon la revendication 9, dans lequel le liant comprend au moins un composé choisi parmi les borates, les phosphates et les silicates minéraux et les substances organiques solubles dans l'eau de masse moléculaire élevée.
